

## UNITED STATES PATENT OFFICE

2,315,347

## COATING COMPOSITION

Walter K. Moffett, South River, N. J., assignor to  
E. I. du Pont de Nemours & Company, Wilming-  
ton, Del., a corporation of Delaware

No Drawing. Application July 12, 1939,  
Serial No. 284,094

8 Claims. (Cl. 260—16)

This invention relates to improved coating compositions and more particularly to cellulose nitrate coating compositions which are highly resistant to discoloration from contact with oils and greases.

Recent advances in the development of cellulose nitrate enamels for automotive and industrial finishing fields and especially for the finishing of automobiles have provided outstanding improvements in general durability and more particularly in the elimination or reduction in chalking tendencies, a deficiency generally encountered in the earlier finishes when exposed to the atmospheric elements. This defect has been largely overcome through the use of special or specially treated pigments on specific types of vehicles. However, in certain instances, these finishes which exhibit superior chalk resistance have proven to be defective in their resistance to "oil spotting" or discoloration when mineral oils or greases are brought in direct contact therewith.

This defect is particularly significant and more frequently encountered in automobile finishes where grease and oil may inadvertently come in contact with the finish from overhead conveyor systems used in assembling the car or during servicing and lubricating of the automobile before or after delivery to the consumer. The new hypoid gear lubricants are quite injurious in this respect. "Oil spotting" is also sometimes caused by the oil-containing rubbing compounds employed in conventional rubbing operations performed after application of the coating composition to bring out high lustre in the finish. Discoloration from this source is particularly apparent when the rubbing compound is permitted to remain on the finish during temporary shutdown periods.

The effect of such oil or grease on the finish is not a softening or destructive action on the film but rather an unsightly discoloration which increases in intensity on exposure to light and which is especially pronounced in the light colored finishes, including "metallic" finishes consisting of low pigmented enamels containing finely ground aluminum, which are generally popular at the present time. The effect seems to be permanent since it cannot be removed by any known cleaning or polishing means without removing excessive amounts of the finish film and, therefore, presents a serious problem in the finishing of surfaces which may be exposed to contact with mineral oils and greases.

This invention, therefore, has as a primary object the provision of a cellulose nitrate coating

composition which affords a finish highly resistant to "oil spotting" or discoloration from contact with mineral oils and greases. Another object of the invention is the provision of a cellulose nitrate coating composition which affords a finish of excellent outdoor durability including superior chalk resistance. A further object is the provision of a cellulose nitrate coating composition which affords a finish that may be readily rubbed and polished. A still further object is the provision of a cellulose nitrate coating composition which affords a finish that is adherent, flexible and substantially non-thermoplastic under a buffering wheel.

These objects are accomplished by means of a composition which is normally non-gelling, comprising cellulose nitrate, certain non-drying vegetable oil modified alkyd resins and an aliphatic dicarboxylic acid.

Some of the aforementioned acids have been proposed as gel inhibitors in cellulose nitrate compositions which normally tend to gel rapidly during shelf storage, particularly in the presence of basic pigments such as zinc oxide. These compositions may include also certain vegetable oil modified alkyd resins which increase gelation tendencies probably because of a high acid number or because they are modified with an oxidizing oil such as linseed oil.

In contradistinction, the present invention is directed to cellulose nitrate compositions which do not normally gel in the complete absence of an inhibiting agent for extended storage periods of a year or more. This is true even when zinc oxide is included in the compositions. The resin ingredient consists of a non-gelling, non-drying vegetable oil modified alkyd resin preferably characterized by an acid number of less than 6 and in any case less than 10. The aliphatic dicarboxylic acids employed in the present invention, therefore, have no effect with respect to inhibiting gelation since no tendency in this direction is apparent even in the complete absence of any inhibiting agent. However, an entirely unexpected and important improvement is now made available through the use of the aforementioned acids for the express purpose of providing a finish which is highly resistant to discoloration from mineral oils and greases, a desirable property which bears no relation whatsoever to gelation tendencies.

The preferred embodiment of the invention is illustrated by the following examples which are not intended to limit the invention except as indicated in the appended claims, since varia-

tions will occur to those skilled in the art without departing from the spirit and scope thereof.

*Example 1*

|                                       | Per cent by weight |
|---------------------------------------|--------------------|
| Cellulose nitrate (low viscosity)     | 15.4               |
| Alcohol (denatured)                   | 5.1                |
| Titanium dioxide                      | 7.0                |
| Butyl acetate                         | 18.7               |
| Methyl ethyl ketone                   | 22.1               |
| Butyl alcohol                         | 3.0                |
| Petroleum naphtha (90-129° C.)        | 4.0                |
| Malic acid solution <sup>1</sup>      | 1.2                |
| Blown castor oil                      | 1.5                |
| Diethyl phthalate                     | 2.3                |
| Synthetic resin solution <sup>2</sup> | 19.7               |
|                                       | 100.0              |

<sup>1</sup> The malic acid solution consisted of a 30% solution of malic acid in denatured ethyl alcohol.

<sup>2</sup> The resin solution of the above example consisted of a mixture of 30 parts of toluol and 70 parts of a synthetic resin which is a reaction product of:

|                    | Per cent |
|--------------------|----------|
| Glycerine          | 16.2     |
| Phthalic anhydride | 36.6     |
| Coconut oil        | 47.2     |
|                    | 100.0    |

This resin was prepared by first heating the glycerine and coconut oil at a temperature between 380 and 400° F. until a homogeneous solution was obtained. The phthalic anhydride was then added and heating continued at about 480° F. until an acid number of 5-6 was obtained. The charge was blanketed with carbon dioxide during the preparation of the resin.

The enamel composition of Example 1 which contains cellulose nitrate, resin, plasticizer and malic acid in the ratio of 10 parts by weight of cellulose nitrate, 9 parts by weight of modified alkyd resin, 2.5 parts by weight of plasticizer, and 0.23 part by weight of malic acid, was prepared by first dispersing the pigment in a cellulose nitrate colloid adjusted to a suitable consistency by the addition of solvents and diluents by a kneading treatment described in U. S. Patent 2,052,470. This pigmented intermediate was then placed in an agitator mixer together with the remaining ingredients including the synthetic resin and malic acid solutions, and the mixture thoroughly agitated until a homogeneous enamel product was obtained.

*Example 2*

|                                       | Per cent by weight |
|---------------------------------------|--------------------|
| Cellulose nitrate (low viscosity)     | 13.1               |
| Ethyl alcohol (denatured)             | 6.9                |
| Chrome yellow pigment                 | 12.0               |
| Isobutyl acetate                      | 14.4               |
| Methyl ethyl ketone                   | 19.5               |
| Petroleum naphtha (90-129° C.)        | 5.1                |
| Ethyl acetate                         | 6.4                |
| Isobutyl alcohol                      | 5.0                |
| Malic acid solution <sup>1</sup>      | 1.0                |
| Castor oil                            | 2.9                |
| Diethyl phthalate                     | 4.3                |
| Synthetic resin solution <sup>2</sup> | 9.4                |
|                                       | 100.0              |

<sup>1</sup> The malic acid solution in this example consisted of a 30% solution of malic acid in denatured ethyl alcohol.

<sup>2</sup> The synthetic resin solution in this example was of the same composition as that described for Example 1.

The enamel composition of Example 2 which contains cellulose nitrate, resin, softener, and malic acid in the ratio of 10 parts by weight

of cellulose nitrate, 5 parts by weight of modified alkyd resin, 3.3 parts by weight of plasticizer and 0.23 part by weight of malic acid, was prepared in accordance with the procedure described for Example 1.

The viscosity characteristic of the cellulose nitrates utilized in the examples was about 3 seconds as determined in accordance with A. S. T. M. Specifications D-301-33T, Formula B.

10 In order to determine whether a finish is resistant to oils and greases an arbitrary test was devised which consists of soaking a felt pad one inch square and  $\frac{1}{8}$  inch in thickness with a heavy automotive transmission oil, preferably a hypoid gear lubricant and placing this oil-soaked pad on the surface of a finished panel for 24 hours at room temperature. The pad is removed and excess oil wiped off with a dry cloth or with a cloth wetted with petroleum naphtha. The 15 finish is then examined for discoloration. A short exposure to direct sunlight seems to accentuate the discoloration if any is present.

The application of this test to finishes prepared by spraying 3 coats suitably thinned of the compositions of Examples 1 and 2 on steel panels primed and surfaced with conventional under-coats failed to show any discoloration whatever, whereas finishes prepared in the same manner with compositions in which no malic acid or equivalent described herein was included and which were otherwise identical with the compositions of Examples 1 and 2 showed serious discoloration.

35 The aliphatic dicarboxylic acids both unsaturated and saturated including hydroxy acids of this class, appear to afford the desired results of markedly reducing or completely eliminating discoloration from oils and greases in the compositions of the present invention. Malic, malonic, maleic, tartaric, adipic, succinic and oxalic are exemplary of the types of acids which have been found suitable. Malic and malonic acids are particularly effective. Phthalic acid, an aromatic dicarboxylic acid, or its anhydride, is also of utility although somewhat less effective than malic or malonic acid.

40 Other methods of dispersing the pigment in the vehicles of the invention may be employed if desired such as by grinding in ball mills, roller mills, burrstone mills or from pigment pulps according to the process described in U. S. Patent 2,140,745.

45 In order to provide a superior enamel which maintains highest chalk resistance combined with resistance to mineral oils and greases when the dicarboxylic acids of the present invention are included and which affords satisfactory working properties, the resin should be modified with from not less than 35% to not more than 60% and preferably with from 40 to 50% of coconut oil or similar non-gelling, nonhydroxy, non-drying oil such as cottonseed or with blown oils of these types. Compositions containing alkyd resins modified with hydroxy oils, such as castor oil, are not preferred in the present invention because of the poor durability and reactivity with reactive type pigments which are imparted to cellulose nitrate coating compositions by such modified resins.

50 In any event, the non-gelling, non-drying oil modified alkyd resin must be prepared so that the acid number is kept as low as possible, preferably not more than 5 or 6 and, in any event, should be kept below 10. Resins of substantially higher acid number have a tendency to gel and also cannot be used with reactive type pigments such as

zinc oxide because of poor stability of the compositions during storage as evidenced by gelling and/or the formation of grit. Such reactive type pigments as referred to in the trade indicate pigments which chemically react with the liquid or solid ingredients in the composition in which they are incorporated.

Optimum resistance to "oil spotting" combined with maximum durability including superior chalk resistance are obtained when the cellulose nitrate-alkyd resin-plasticizer ratios and the amount of dicarboxylic acid employed are kept within definite limits. These ratios should be such that for each 10 parts by weight of cellulose nitrate, the amount of alkyd resin is kept below 10 parts but not less than about 5 parts. If the proportion of alkyd resin to cellulose nitrate is increased by a small amount as, for instance, to 1 part of alkyd resin to 1 part of cellulose nitrate, the compositions while possibly useful for some industrial purposes even with somewhat higher proportions of the modified alkyd resin, are of no value practically for the present primary purpose of finishing automobiles because the conventional sanding, rubbing and polishing operations employed in this industry cannot be satisfactorily practiced. The amount of plasticizer is about 2 parts when the maximum quantity of resin is used and about 5 parts when the minimum amount of resin is used.

These acids are preferably incorporated in an amount between 0.2% and 2.0% based on the total weight of the composition to be treated. In most cases an amount of between 0.2% and 0.6% is quite effective, particularly in the case of the more preferred acids, namely, malic acid and malonic acid. Excessive proportions are to be avoided since in such cases there may be a tendency for the acid to exude on the surface of the finish in the form of a whitish deposit, thus adversely affecting the original gloss and beauty of the finish.

Cellulose nitrate with a viscosity characteristic on the order of that indicated in the examples is preferred, but the use of commercially available cellulose nitrates of still lower or higher viscosities is not precluded since the several advantages hereinafter described likewise accrue.

The solvents and diluents shown in the examples are, of course, merely illustrative of a large number of such materials well known and widely used in the art, and many other equivalent materials may be satisfactorily substituted therefor. Suitable solvents and diluents include esters of lower fatty acids, for example, ethyl acetate, butyl acetate, amyl acetate, isobutyl acetate, butyl propionate and the like, ketones such as methyl ethyl ketone, alcohol ethers and their esters, such as ethylene glycol monoethyl ether acetate and ethylene glycol monomethyl ether acetate, lower aliphatic alcohols and aliphatic and aromatic hydrocarbon diluents such as petroleum naphtha and toluene.

The plasticizers and softeners which may be employed in the compositions of the present invention include conventional materials such as castor oil, blown castor oil, aryl sulfonamides including ortho, meta and para tolueen ethyl sulfonamides and mixtures of these, aryl and alkyl esters of phosphoric acid, dibutyl tartrate, di-cyclohexyl phthalate, diethyl phthalate and the phthalate esters of ether alcohols, such as the phthalate ester of ethylene glycol monomethyl ether.

The invention is operative for cellulose nitrate-

non-gelling, non-hydroxy, non-drying vegetable oil modified alkyd resin compositions which include the commonly used pigments or other coloring matter such as antimony oxide, titanium dioxide, titanate pigments, iron blue pigments, chrome pigments, para and toluidine toners, maroons, carbon black, ultramarine blue, burnt umber, iron oxide, etc. If zinc oxide, a basic type pigment, is employed to any considerable extent in the compositions of the present invention, little if any improvement in resistance to oil-spotting is obtained by the use of the above described dicarboxylic acids which are otherwise so outstandingly effective. The invention is particularly valuable when employed with the light colored so-called pastel shade and metallic enamels which have been a considerable source of complaint in the previously available enamels because of poor resistance to oils and greases where discoloration is more pronounced.

Although phthalic anhydride is the preferred acid radical in the alkyd resin ingredient of the improved compositions, other acids such as succinic, malic, adipic, maleic, sebacic, etc., may be substituted wholly or in part for the phthalic anhydride, but best results are secured when phthalic anhydride is present in preponderant proportions.

Suitable resins for the improved compositions may also be prepared using other polyhydric alcohols including ethylene glycol and higher homologs, diethylene glycol and other polyglycols; polyglycerols; pentaerythritol and sorbitol.

The compositions of the invention are generally useful in finishing surfaces which may be exposed to direct contact with oils and greases. They are particularly useful for finishing automobiles where contact with lubricating oils and greases and oil-containing rubbing compounds is more frequently encountered.

The new compositions have shown a number of important advantages when employed in the suggested utilities. In the first place, they have exhibited an unexpected and decisively superior resistance to spotting or discoloration of the finish from "oily" rubbing and polishing compounds and from direct contact with oils and greases which sometimes reach the finish of an automobile through careless servicing of the car before or after delivery to the customer. This defect of "oil spotting" was quite common in commercial finishes heretofore available and caused frequent consumer complaint and costly rejections in the final inspection in the manufacture of new automobiles. Furthermore, the new compositions are adherent and flexible and afford excellent durability, including superior resistance to chalking, thus preserving the original gloss and lustre for extended periods during exposure to atmospheric conditions. The enamels of the present invention provide finishes of satisfactory working properties which do not become thermoplastic or soften under the rubbing and polishing operations normally practiced in the automotive industry. The satisfactory working properties of the improved compositions as controlled by the particular proportions previously indicated are of considerable importance inasmuch as previously known compositions containing related ingredients are usually quite defective in this respect, making them entirely unsuited for the present purpose. Substantial economies are represented in the new finishes in that assembly line rejections and consumer complaints necessitating

75 "touching up" or refinishing of automobiles be-

cause of "oil spotting" discoloration are practically eliminated.

As many widely different embodiments of the invention may be made without departing from the spirit and scope thereof, it will be understood that the invention is not limited to the specific embodiments thereof except as defined in the appended claims.

I claim:

1. A coating composition which is highly resistant to oils and greases consisting of (A) a normally non-gelling coating composition containing cellulose nitrate and a non-gelling, non-hydroxy, non-drying vegetable oil modified alkyd resin characterized by an acid number of less than 10 and (B) in addition thereto an aliphatic dicarboxylic acid in the proportions of between 0.2 and 2.0% by weight of the total coating composition.

2. Composition of claim 1 in which the aliphatic dicarboxylic acid is malic acid.

3. Composition of claim 1 in which the aliphatic dicarboxylic acid is malonic acid.

4. The composition of claim 1 in which the alkyd resin is modified with from 35 to 60 per cent of the non-hydroxy, non-drying vegetable oil.

5. Composition of claim 1 in which the alkyd resin is modified with coconut oil.

6. Composition of claim 1 in which said modified alkyd resin is a glycercyl phthalate resin.

5 7. Composition of claim 1 in which the aliphatic dicarboxylic acid is present in an amount of about 0.5% by weight of the total coating composition.

8. A normally non-gelling, weather-resistant 10 cellulose nitrate coating composition which is highly resistant to oils and greases consisting of (A) a normally non-gelling composition containing cellulose nitrate, a plasticizer, an alkyd resin modified with 35-60% of a non-hydroxy, non-drying vegetable oil, said resin having an acid 15 number of less than 10 and being present in said composition in a proportion by weight of at least 5 parts as a minimum but less than 10 parts as a maximum for each 10 parts of cellulose nitrate, said plasticizer being present in the proportion by weight of about 2 parts as a minimum and 5 parts as a maximum and (B) in addition thereto an aliphatic dicarboxylic acid in the proportion of between 0.2 and 2.0% by weight of the 20 25 total coating composition.

WALTER K. MOFFETT.